

# United States Patent Office

3.443.953

Patented May 13, 1969

1

**3,443,953**  
**PHOTOGRAPHIC MATERIALS FOR THE SILVER**  
**DYESTUFF BLEACHING PROCESS**  
Hansrolf Loeffel, Bern, Switzerland, assignor to Ciba  
Limited, Basel, Switzerland, a Swiss Company  
No Drawing. Filed Nov. 30, 1965, Ser. No. 510,672  
Claims priority, application Switzerland, Dec. 2, 1964  
15,506/64  
Int. Cl. G03c 1/10

U.S. Cl. 96—99 Int. Cl. G03E 17/10 6 Claims

## 6 Claims

#### ABSTRACT OF THE DISCLOSURE

Photographic materials for the silver dyestuff bleaching process. These materials are characterized in that they contain on a support a layer containing silver halide and at least one yellow dyestuff of the formula



in which  $R_1$  and  $R_1'$  each represents a benzene or a naphthalene radical containing at least one sulfonic acid group,  $R_2$  and  $R_2'$  each represents a benzene or a naphthalene radical bound in 1,4-position to the  $-\text{N}=\text{N}-$  group and the  $-\text{NH}-\text{OC}-$  group and  $R_3$  and  $R_3'$  each represents a benzene radical. These yellow dyestuffs are fast to diffusion, stable during drying and storage and easy to bleach.

are advantageously used, in which  $R_4$  represents a benzene or a naphthalene residue containing at least two sulphonic acid groups,  $R_5$  represents a benzene or a naphthalene residue bound in 1,4-position to the  $-\text{N}=\text{N}-$  group and the  $-\text{NH}-\text{OC}-$  group and  $R_6$  represents a monocyclic benzene residue.

The residue  $R_1$  or  $R_4$  may be a benzene residue substituted by two sulphonate groups and which contains at most an alkyl group, for example, a methyl group as a further substituent. The said residue may also be a naphthalene residue substituted by two sulphonate groups and which does not contain further substituents.  $R_2$  and  $R_5$  is a naphthalene or, preferably, a benzene residue which is bound in 1,4-position to the  $-\text{N}=\text{N}-$  and  $-\text{NH}-\text{CO}-$  groups. When a naphthalene residue is present it may be unsubstituted or may contain a sulphonate group advantageously in a  $\beta$ -position of the six-membered ring not bound to the  $-\text{N}=\text{N}-$  group. When  $R_2$  or  $R_5$  is a benzene residue it may contain as substituents, for example, one or two alkyl groups or a hydroxalkoxy group, an alkoxy group or an acylamino group, and no further substituents in addition to the two last-mentioned groups, or an alkyl group. All these substituents advantageously contain not more than four carbon atoms.

Accordingly, the layer dyestuffs may advantageously correspond to one of the formulae

(3)



and (4)



The present invention provides photographic materials for the silver dyestuff bleaching process, which materials contain on a support a layer containing at least one dye-stuff of the formula

in which  $R_6$  preferably represents a benzene residue,  $X$  represents a hydrogen atom or an alkyl, alkoxy or an acylamino group advantageously derived from a low-molecular weight fatty acid,  $Y$  represents a hydrogen atom or an alkyl group and  $m$  and  $n$  each represents an integer not greater than 2.

50 atom or an alkyl group and  $m$  and  $n$  each represents an integer not greater than 2.

68



in which  $R_1$  and  $R_1'$  each represents a benzene or a naphthalene residue containing at least one sulphonic acid group,  $R_2$  and  $R_2'$  each represents a benzene or a naphthalene residue bound in 1,4-position to the  $-\text{N}=\text{N}-$  group and the  $-\text{NH}-\text{OC}-$  group and  $R_3$  and  $R_3'$  each represents a monocyclic residue having 5 to 6 ring members.

## Symmetrical dyestuffs of the formula

$$(2) \quad \begin{array}{c} R_4-N=N-R_5-NH-OC-R_6- \\ \qquad \qquad \qquad | \\ \qquad \qquad \qquad N=N-R_6-CO-HN-R_5-N=N-R_4 \end{array}$$

in which X and Y have the meanings given above

The trisazo dyestuffs of the Formula 1 can be prepared from aminoazo dyestuffs of the formula

65 (6)  $R_1-N=N-R_2-NH_2$   
 in which  $R_1$  and  $R_2$  have the meanings given above, these  
 aminoazo dyestuffs being obtained by coupling a diazo-  
 tized aminobenzene sulphonic acid or aminonaphthalene  
 70 disulphonic acid with an aminobenzene or aminonaph-  
 thalene capable of coupling in para-position to the amino-  
 group. When an aminoazo dyestuff of the Formula 6

is reacted in a molecular ratio of 2:1 with a dihalide, preferably the dichloride, of an azobenzene- or azothiophene-dicarboxylic acid of the formula



symmetrical trisazo dyestuffs are obtained. The residues  $\text{R}_3$  and  $\text{R}'_3$  in the Formula 1 and the Formula 7 are monocyclic and thus contain a single benzene ring without any further rings connected therewith, either simply or by anellation.

The following compounds may be mentioned as starting materials from which the trisazo dyestuffs can be prepared in the manner indicated above:

Diazo components

1-aminobenzene-2,4-disulphonic acid,  
1-aminobenzene-2,5-disulphonic acid,



1-amino-4-methylbenzene-2,5-disulphonic acid,  
1-aminonaphthalene-3,6-disulphonic acid,  
2-amino-naphthalene-4,8-disulphonic acid,  
2-aminonaphthalene-3,6-disulphonic acid,  
2-aminonaphthalene-5,7-disulphonic acid,  
2-aminonaphthalene-6,8-disulphonic acid,  
2-aminonaphthalene-4,6,8-trisulphonic acid,  
2-aminonaphthalene-3,6,8-trisulphonic acid,  
2-aminonaphthalene-1,5,7-trisulphonic acid.

Coupling components

1-amino-2- or 3-methylbenzene, 1-amino-2,5- or 2,6-dimethylbenzene, 1-amino-2- or 3-methoxybenzene, 1-amino-2- $\beta$ -hydroxyethoxybenzene, 1-amino-2-methoxy-5-methylbenzene, 1-amino-3-acetylaminobenzene, 3-amino-phenylurea, 1-aminobenzene- $\omega$ -methanesulphonic ester, 1-amino-2- or 3-ethoxybenzene, 1-amino-2- or 3- $\beta$ -hydroxyethoxybenzene, 1-amino-2- $\beta$ -hydroxy-5-methylbenzene, 1-amino-2-methoxy-5-methylbenzene, 1-amino-2,5-dimethoxybenzene, 1-amino-2-ethoxy-5-methylbenzene, 1-amino-2-chloro-5-methoxybenzene, 3-amino-4-methyl-phenoxyacetic acid, 1-aminonaphthalene-5-sulphonic acid.

Dicarboxylic acids

Azobenzene-3,3'-dicarboxylic acid,  
4,4'-dimethylazobenzene-3,3'-dicarboxylic acid,  
4,4'-dichloroazobenzene-3,3'-dicarboxylic acid,  
azobenzene-4,4'-dicarboxylic acid,  
2,2'-dimethylazobenzene-5,5'-dicarboxylic acid,  
2,2'-dimethoxyazobenzene-5,5'-dicarboxylic acid,  
2,2'-dichloroazobenzene-5,5'-dicarboxylic acid,  
2,2'-dimethylazobenzene-4,4'-dicarboxylic acid,  
3,3'-dichloroazobenzene-4,4'-dicarboxylic acid,  
4,4'-dichloroazobenzene-5,5'-dicarboxylic acid,  
2,2'-azothiophene-5,5'-dicarboxylic acid.

The dyestuffs of the Formulae 1 to 5 can be prepared by known methods. Coupling to form the aminomonoazo dyestuffs is carried out in an acid medium.

Amines difficult to couple may be coupled in the form of their  $\omega$ -methanesulphonic acids, with subsequent elimination of the methanesulphonic acid group. The amino-azo dyestuffs are advantageously reacted with the dicarboxylic acid halide containing azo groups in the presence of an agent capable of binding acid. Like the dyestuffs themselves, the photographic layers containing, in accordance with the invention, at least one dyestuff of the Formula 1 may also be prepared by known methods and used for the production of colored images. In particular,

the dyestuffs of the Formula 1 may be present in multi-layer material containing on a support a red-sensitized layer dyed with a cyan dyestuff, a green-sensitized layer dyed with a magenta dyestuff and, finally, a blue-sensitized layer dyed with a dyestuff of the Formula 1.

5 The dyestuffs of the Formula 1 are generally very resistant to diffusion in the usual kinds of layer. They display no tendency to change into an opalescent or dull form in the gelatine layers during drying and storage, and they are easily reduced to harmless and/or easily 10 water-extractable decomposition products in the dyestuff bleaching bath.

The following examples illustrate the invention. Unless otherwise stated, the parts and percentages are by weight.

15

EXAMPLE 1

12 milligrams of the dyestuff of the formula



are dissolved at 70° C. in 2 cc. of distilled water. The solution is cooled to 40° C. and added to 3.5 cc. of a 6% aqueous gelatine at 40° C. 3.3 cubic centimetres of a 30 gelatine silver bromide emulsion at a temperature of 40° C. are then added. If necessary, 1 to 2 cc. of an aqueous solution of a dispersing agent, for example, saponin, and a hardening agent, for example, dimethylolurea, are added. The mixture so prepared is cast on a glass plate 35 measuring 13 cm.  $\times$  18 cm. and dried.

The film is exposed behind a step-wedge and the silver image is developed in a 1-methylamino-4-hydroxybenzenesulphate hydroquinone developer and fixed.

The image dyestuff is then bleached out depending on 40 the amount of silver present, in a bath containing 30 to 100 parts by volume of 32% hydrochloric acid, 40 to 120 parts of potassium bromide, 30 to 50 parts of thiourea and 0.001 to 0.01 part of 2-amino-3-hydroxyphenazine per 1,000 parts by volume. Subsequently, excess silver is removed in a bath containing 100 parts of sodium chloride, 100 parts of copper sulphate crystals and 50 parts by volume of 37% hydrochloric acid per 1,000 parts by volume. Fixation is then carried out in the usual manner. A yellow image which is the inverse of the silver wedge is obtained which is bleached pure white at the 45 areas where the silver was present in the greatest density. A yellow image of this kind can also form part of multi-colour photographic material; in this case, the amounts of gelatine are adapted to suit the required thickness of the layers.

50 The dyestuff of the Formula 8 may be prepared as follows:

60.6 parts of 2-aminonaphthalene-4,8-disulphonic acid, in the form of the sodium salt, are dissolved in 1,000 parts of water, the solution is cooled with ice to 0° C., and 60 diazotized in the usual manner with 65 parts of 37% hydrochloric acid and 14 parts of sodium nitrite. 30.5 parts of 2-methoxy-5-methyl-1-aminobenzene are dissolved at 65 60 to 70° C. in 300 parts of water and 30 parts of 37% hydrochloric acid, the solution is cooled with ice to 5° C. and added to the solution of the diazo compound. The 70 batch is stirred for 24 hours at a temperature of 8 to 15° C. to complete the coupling time and can be shortened by buffering the mineral acid with sodium acetate. The acidic suspension of the monoazo dyestuff is heated to 65° C. and is then filtered at 30° C.

6 parts of the aminomonoazo dyestuffs so obtained are dissolved in 150 parts of water and then 5.2 parts of sodium borate are added to the solution at room temperature. 2 parts of azobenzene-4,4'-dicarboxylic acid dichloride are dissolved in 50 parts by volume of warm acetone,

and the solution so obtained is added all at once to the solution of the aminoazo dyestuff. The reaction mixture is stirred for 12 to 14 hours at room temperature and is then heated to 60° C. and kept at that temperature for one hour. The trisazo dyestuff so formed is precipitated by the addition of 300 parts by volume of ethanol and 100 parts by volume of 7 N potassium acetate and is then isolated by suction filtration. Purification is effected by dissolving the dyestuff in 200 parts of water, precipitating it by the addition of 50 parts by volume of ethanol and 100 parts by volume of 7 N potassium acetate, and again isolating it by suction filtration. After drying, about 4 parts of dyestuff are obtained.

The azobenzene-4,4'-dicarboxylic acid dichloride can be prepared in the following manner:

93 parts of zinc dust are added during 20 minutes to a mixture of 100 parts of para-nitrobenzoic acid, 700 parts of water and 400 parts by volume of 30% sodium hydroxide solution, during which process the temperature rises to 60° C. The reaction mixture is heated from 90 to 95° C., which causes it to thicken, and then 500 parts of water are added. The batch is stirred for 12 hours at 90° C.

The reaction mixture is then discharged into 10,000 parts of hot water whereby the azobenzene dicarboxylic acid dissolves. After purification by filtration, 25 parts of

sodium hypochlorite solution containing 13 to 14% of active chlorine are added to the filtrate. 320 parts by volume of glacial acetic acid are added and the dicarboxylic acid precipitates. After one hour the batch is suction filtered and the filter cake is washed with 500 parts of 1% acetic acid and with 500 parts of water. The residue is dried in vacuo and 74 parts of azobenzene-4,4'-dicarboxylic acid are obtained in the form of a pink powder.

54 parts of azobenzene-4,4'-dicarboxylic acid, 200 parts of phosphorus pentachloride, 1,420 parts by volume of orthodichlorobenzene and 5 parts of dimethyl formamide are heated to 150° C. and kept at that temperature for 20 minutes. The batch is allowed to cool to 80° C. and about half the amount of dichlorobenzene is distilled off in vacuo. The batch is allowed to cool overnight and the azobenzene-4,4'-dicarboxylic acid dichloride precipitates in the form of red crystals. The batch is filtered and the residue is washed with benzene and dried in vacuo at 50° C. 43 parts of acid chloride melting at 157 to 159° C. are obtained.

Any one of the dyestuffs II to XIX obtainable from the components listed in the following table may be incorporated in a gelatine layer in the manner indicated instead of the dyestuff of the Formula 8. These dyestuffs may be prepared in a manner analogous to that used for the dyestuff of the Formula 8.

| Dyestuff No.     | Diazo component | Coupling component | Condensation component | Absorp-<br>tion<br>max.,<br>$\mu\mu$ |
|------------------|-----------------|--------------------|------------------------|--------------------------------------|
| I (=Formula [S]) |                 |                    |                        | 436                                  |
| II               |                 |                    |                        | 430                                  |
| III              |                 |                    |                        | 400                                  |
| IV               |                 |                    |                        | 400                                  |
| V                |                 |                    |                        | 434                                  |
| VI               |                 |                    |                        | 410                                  |

| Dyestuff No. | Diazo component | Coupling component | Condensation component | Absorp-<br>tion<br>max.,<br>m.<br>$\mu$ |
|--------------|-----------------|--------------------|------------------------|-----------------------------------------|
| VII          |                 |                    |                        | 430                                     |
| VIII         |                 |                    |                        | 430                                     |
| IX           |                 |                    |                        | 415                                     |
| X            |                 |                    |                        | 400                                     |
| XI           |                 |                    |                        | 424                                     |
| XII          |                 |                    |                        | 412                                     |
| XIII         |                 |                    |                        | 408                                     |
| XIV          |                 |                    |                        | 412                                     |
| XV           |                 |                    |                        | 308                                     |

| Dyestuff No. | Diazo component | Coupling component | Condensation component | Absorp-<br>tion<br>max.,<br>$m\mu$ |
|--------------|-----------------|--------------------|------------------------|------------------------------------|
| XVI          |                 |                    |                        | 400                                |
| XVII         |                 |                    |                        | 400                                |
| XVIII        |                 |                    |                        | 420                                |
| XIX          |                 |                    |                        | 420                                |

## EXAMPLE 2

The following layers are applied in the sequence indicated to a white, opaque acetate film provided with an adhesive layer:

(1) A red-sensitized silver bromide emulsion in gelatine containing the cyan dyestuff of the formula

(9)



(2) A colorless gelatine layer containing no silver halide.

(3) A green-sensitized silver bromide emulsion in gelatine containing the magenta dyestuff of the formula

(10)



(4) A yellow filter layer containing the dyestuff of the formula

(11)



(5) A blue-sensitized silver bromide emulsion in gelatine containing the yellow dyestuff of the Formula 8.

The gelatine layers may contain additives, for example, wetting agents, hardeners and stabilizers for the silver halide. The material is manufactured in a manner such that each layer (except (2)) contains, per square metre

35 of film, 0.5 gram of dyestuff and a quantity of silver bromide corresponding to 1 to 1.2 grams of silver.

The film so prepared is exposed to red, green and blue light beneath a coloured diapositive. The reproduction is then developed in the following manner:

40 (1) Developing for 6 minutes in a bath containing,

(9)



50 per litre, 50 grams of anhydrous sodium sulphate, 0.2 gram of 1-phenyl-3-pyrazolidone, 6 grams of hydroquinone, 35 grams of anhydrous sodium carbonate, 4 grams of potassium bromide and 0.3 gram of benztriazole.

(10)



(2) Washing with water for 5 minutes.

(3) Fixing for 6 minutes in a solution of 200 grams of sodium thiosulphate crystals and 20 grams of potassium metabisulphite in 1 litre of water.

(4) Washing with water for 5 minutes.

(5) Dyestuff bleaching for 3 to 12 minutes with a solution containing, per litre of water, 50 to 80 grams of potassium bromide, 40 to 80 grams of thiourea, 35 to 80 grams of 30% sulphuric acid and, if desired, 0.01 gram of 2-amino-3-hydroxyphenazine.

(6) Washing with water for 10 minutes.

(7) Bleaching residual silver for 5 minutes with a solution containing 60 grams of copper sulphate crystals, 80 grams of potassium bromide and 15 ml. of 30% hydrochloric acid per litre of water.

75

- (8) Washing with water for 5 minutes.  
 (9) Fixing for 5 minutes in the manner described under 3.  
 (10) Washing with water for 5 minutes.  
 A true, positive image to be viewed in incident light and which is fast to light and otherwise permanent is obtained.



It is also possible to use the dyestuffs II to XIX instead of the dyestuff of the Formula 8.

What is claimed is:

1. Photographic material for the silver dyestuff bleaching process which contains on a support a layer containing silver halide and at least one dyestuff of the formula 20



in which  $R_1$  and  $R_1'$  each represents a radical selected from the group consisting of benzene and naphthalene containing at least one sulphonate acid group,  $R_2$  and  $R_2'$  each represents a radical selected from the group consisting of benzene and naphthalene bound in 1,4-position to the  $-N=N-$  group and the  $-NH-OC-$  group and  $R_3$  and  $R_3'$  each represents a benzene radical.

2. Photographic materials as claimed in claim 1, where-



in the layer contains silver halide and a dyestuff of the formula



in which  $R_4$  represents a radical selected from the group consisting of benzene and naphthalene containing at least two sulfonic acid groups,  $R_5$  represents a radical selected



from the group consisting of benzene and naphthalene bound in 1,4-position to the  $-N=N-$  group and the  $-NH-OC-$  group and  $R_6$  represents a benzene radical.

3. Photographic material as claimed in claim 1 in which the layer contains silver halide and a dyestuff of the formula



in which  $R_6$  represents a radical selected from the group consisting of benzene and thiophene,  $X$  represents a member selected from the group consisting of a hydrogen atom, an alkyl group, and an alkoxy group,  $Y$  represents a member selected from the group consisting of a hydrogen atom and an alkyl group, and  $m$  and  $n$  each represents an integer of at the most 2.

4. Photographic material as claimed in claim 1, in which the layer contains silver halide and a dyestuff of the formula



in which  $R_6$  represents a benzene radical,  $X$  represents a member selected from the group consisting of a hydrogen atom, an alkyl group, and an alkoxy group and  $Y$  represents a member selected from the group consisting of a hydrogen atom and an alkyl group.

5. Photographic material as claimed in claim 4, in which the layer contains silver halide and a dyestuff of the formula



in which  $X$  represents a member selected from the group consisting of a hydrogen atom, an alkyl, and an alkoxy and  $Y$  represents a member selected from the group consisting of a hydrogen atom and an alkyl group.

6. Photographic material as claimed in claim 5, in which the layer contains silver halide and the dyestuff of the formula:



#### References Cited

#### UNITED STATES PATENTS

2,286,714 6/1942 Chechak ----- 96-99

J. TRAVIS BROWN, Primary Examiner.

U.S. Cl. X.R.

96-20; 260-169